

## UNITED STATES PATENT OFFICE

2,223,129

## LUBRICANT

Carl F. Prutton, East Cleveland, Ohio, assignor to  
The Lubri-Zol Corporation, Wickliffe, Ohio, a  
corporation of Ohio

No Drawing. Application May 1, 1940,  
Serial No. 332,782

26 Claims. (Cl. 252—32)

This invention relates, as indicated, to lubricating compositions and more particularly to lubricating compositions which are predominantly hydrocarbon oil, the properties of which affecting its use for particular purposes are improved by the addition of materials which are particularly effective in rendering the lubricants suitable for use under conditions of extreme stress as imposed by high temperatures, high loads, etc.

10 In my co-pending applications, Ser. Nos. 737,070, filed July 26, 1934; 216,153, filed June 27, 1938; and 245,226 filed December 12, 1938, I have disclosed a broad class of lubricating compositions of general utility, particularly in the field 15 of use where extreme pressures are encountered.

My present invention relates to the discovery that a certain class of such materials is particularly suitable for use in lubricants subjected to conditions of extreme stress such as those involved in the lubrication of heavily loaded gears, and in the lubrication of internal combustion engines operating under severe service conditions; for example, those encountered by internal combustion engines particularly of the aviation and 25 Diesel types.

It is the principal object of my invention, therefore, to provide a lubricating composition which is especially suited for the purposes described.

Other objects of my invention will appear as 30 the description proceeds.

To the accomplishment of the foregoing and related ends, said invention, then, consists of the means hereinafter fully described and particularly pointed out in the claims; the following 35 description setting forth in detail certain approved combinations of ingredients embodying my invention, such disclosed means constituting, however, but one of various forms in which the principle of the invention may be used.

40 Broadly stated, this invention comprises the provision of a lubricating composition for the purposes specified, characterized by the fact that the same contains a lubricating oil, preferably of the hydrocarbon type, as a major constituent with the properties of such composition affecting 45 its use as a lubricant, especially under the conditions specified, by the incorporation therein of a minor amount, based on the amount of lubricating oil present, of a stable, oil-soluble salt of 50 an aromatic acid.

More especially, my invention comprises the discovery that salts of aromatic acids, of the type which contain a substituent selected from the class consisting of aliphatic and cyclo-aliphatic radicles, are particularly suited for use.

## THE OIL BASE

The oil base of my lubricating compositions is a lubricating oil of the type best suited for the particular use for which the ultimate composition is designed. When the lubricating compositions of my invention are designed for the lubrication of automobiles, the oil base will of course preferably consist of a refined mineral lubricating oil of lubricating viscosity for the particular point of application. In other words, a conventional gear oil may be used for the lubrication of the gears and generally a lighter, more highly refined, oil will be used in the crank case.

5 This invention is applicable to lubricating compositions in which the base may consist either entirely or in part of synthetic oils, hydrogenated oils, and volatilized oils.

10 The oil base may also desirably contain other well known constituents such as those which improve the oiliness, pour point, cold test, and oxidation properties, etc., of the oil. In general, compositions of my invention may be employed with any commercially available addition agents 15 for the above defined purposes since they are 20 generally compatible with the same in the amounts usually used.

## THE ADDITION AGENTS

25 As above indicated, the addition agents may be generally defined as salts of aromatic acids. The term salts as used herein is intended to include the organic salts of aromatic acids as well as the inorganic salts of aromatic acids. The 30 inorganic salts such as the metallic salts of aromatic acids will generally be found to give best results, and of these, those salts in which the metal is present in divalent form, will usually be 35 preferred.

40 The halogen bearing salts of aromatic acids generally are a broad class of addition agents which have been found to be notably effective.

45 For certain uses, the salts of aromatic acids of the type which contain a substituent selected from the class consisting of aliphatic radicles and cyclo-aliphatic radicles have been found very useful. This latter class of salts may optionally also contain a halogen such as chlorine.

50 Due to the nature of the addition agents contemplated for use, they may be conveniently identified by first having reference to the various aromatic acids from which the salts may be prepared and by then giving a list of the various radicles or bases which may be combined 55 with such acids in producing the salts.

In the following table will be found listed a number of aromatic acids.

TABLE I.—*Aromatic acids*

|    |                                                                                                                                                                                                                                                                                   |
|----|-----------------------------------------------------------------------------------------------------------------------------------------------------------------------------------------------------------------------------------------------------------------------------------|
| 5  | Benzoic acid                                                                                                                                                                                                                                                                      |
| 5  | Benzoic acid derivatives:                                                                                                                                                                                                                                                         |
|    | Azobenzolic acid                                                                                                                                                                                                                                                                  |
|    | Mercapto benzoic acid                                                                                                                                                                                                                                                             |
|    | Alkylated benzoic acids:                                                                                                                                                                                                                                                          |
|    | Lauryl benzoic acid                                                                                                                                                                                                                                                               |
| 10 | Salicylic acid                                                                                                                                                                                                                                                                    |
|    | Salicylic acid derivatives:                                                                                                                                                                                                                                                       |
|    | Alkylated salicylic acids:                                                                                                                                                                                                                                                        |
|    | Ethyl salicylic acid                                                                                                                                                                                                                                                              |
|    | Heterocyclic acids:                                                                                                                                                                                                                                                               |
| 15 | Pyrrole carboxylic acid                                                                                                                                                                                                                                                           |
|    | Thiophene carboxylic acid                                                                                                                                                                                                                                                         |
|    | Acetic acid derivatives:                                                                                                                                                                                                                                                          |
|    | Phenyl acetic acid                                                                                                                                                                                                                                                                |
|    | Diphenyl acetic acid                                                                                                                                                                                                                                                              |
| 20 | Stearic acid derivatives:                                                                                                                                                                                                                                                         |
|    | Phenyl stearic acid                                                                                                                                                                                                                                                               |
|    | Phenyl mercapto stearic acid                                                                                                                                                                                                                                                      |
|    | Xenyl stearic acid                                                                                                                                                                                                                                                                |
| 25 | Naphthyl stearic acid                                                                                                                                                                                                                                                             |
|    | Tolyl stearic acid                                                                                                                                                                                                                                                                |
|    | Puroic acid                                                                                                                                                                                                                                                                       |
|    | Cinnamic acid                                                                                                                                                                                                                                                                     |
|    | Phthalic acid                                                                                                                                                                                                                                                                     |
| 30 | Tuloic acid                                                                                                                                                                                                                                                                       |
|    | Mercapto rosolic acid                                                                                                                                                                                                                                                             |
|    | Naphthyoic acid                                                                                                                                                                                                                                                                   |
|    | Any of the corresponding thio acids.                                                                                                                                                                                                                                              |
|    | Any of the foregoing which have been halogenated.                                                                                                                                                                                                                                 |
| 35 | In the preparation of those salts of aromatic acids of the type in which the aromatic acid is of the class which contains a substituent selected from the class consisting of aliphatic radicles and cyclo-aliphatic radicles, such acids may be conveniently prepared either by: |
|    | (1) Condensing an aromatic compound with                                                                                                                                                                                                                                          |
|    | (a) An aliphatic unsaturated acid, or                                                                                                                                                                                                                                             |
|    | (b) A halogenated aliphatic acid, or                                                                                                                                                                                                                                              |
| 45 | (c) A cyclo-aliphatic unsaturated acid, or                                                                                                                                                                                                                                        |
|    | (d) A halogenated cyclo-aliphatic acid; or by                                                                                                                                                                                                                                     |
|    | (2) Condensing an aromatic acid with                                                                                                                                                                                                                                              |
|    | (a) An unsaturated aliphatic compound, or                                                                                                                                                                                                                                         |
| 50 | (b) A halogenated aliphatic compound, or                                                                                                                                                                                                                                          |
|    | (c) An unsaturated cyclo-aliphatic compound, or                                                                                                                                                                                                                                   |
|    | (d) A halogenated cyclo-aliphatic compound.                                                                                                                                                                                                                                       |
| 55 | In the table below will be found listed examples of aromatic compounds which may be used in any of the condensation reactions identified under Table I above in the preparation of aromatic acids from which appropriate salts may be prepared:                                   |

TABLE II.—*Aromatic compounds*

|    |                   |
|----|-------------------|
|    | Benzene           |
|    | Naphthalene       |
|    | Toluene           |
| 65 | Ethylbenzene      |
|    | Xylene            |
|    | Mesitylene        |
|    | Chlorbenzene      |
|    | Dichlorbenzene    |
| 70 | Chlor-naphthalene |
|    | Chlortoluene      |
|    | Diphenyl          |
|    | Chlordiphenyl     |
|    | Retene            |
| 75 | Chlor-retene      |

The following is a list of aliphatic unsaturated acids which may be used as one of the components of the condensation reactions identified under (1) (a) above in the preparation of aromatic acids from which salts may be accordingly prepared.

TABLE III.—*Aliphatic unsaturated acids*

|                     |    |
|---------------------|----|
| Vinyl acetic acid   | 10 |
| Vinyl acrylic acid  |    |
| Vinyl glycolic acid |    |
| Acrylic acid        |    |
| Crotonic acid       |    |
| Oleic acid          |    |
| Linolenic acid      | 15 |
| Maleic acid         |    |
| Fumaric acid        |    |
| Linoleic acid       |    |
| Elaeostearic acid   |    |
| Propiolic acid      | 20 |
| Stearolic acid      |    |
| Methyl acrylic      |    |
| Beta pentanoic acid |    |
| Undecylenic         |    |
| Myristolenic        | 25 |
| Palmitolenic        |    |

In the following table are given a number of representative examples of halogenated aliphatic acids which may be used in the condensation reactions identified under I above.

TABLE IV.—*Halogenated aliphatic acids*

|                                                                                |    |
|--------------------------------------------------------------------------------|----|
| Chlorstearic acid                                                              | 35 |
| Chloracetic acid                                                               |    |
| Chlorlauric acid                                                               |    |
| Chlorpalmitic acid                                                             |    |
| Dichloroleic acid                                                              |    |
| Chlorbutyric acid                                                              |    |
| Chlorricinoleic acid                                                           |    |
| Chlorlactic acid                                                               | 40 |
| Chlorcitic acid                                                                |    |
| Chlorsuccinic acid                                                             |    |
| Chlormyristic acid                                                             |    |
| As well as the chlor derivatives of all of the acids given in Table III above. | 45 |

In the following table are given representative examples of cyclo-aliphatic unsaturated acids which may be used as one component of the condensation reaction identified under (1) (b) above.

TABLE V.—*Cyclo-aliphatic unsaturated acids*

|                   |
|-------------------|
| Chaulmoogric acid |
| Hydrocarpic acid  |

In the following table are given certain representative examples of halogenated cyclo-aliphatic acids which may be used as one of the components of the condensation reaction referred to under (1) (c) above.

TABLE VI.—*Halogenated cyclo-aliphatic acids*

|                              |    |
|------------------------------|----|
| Chlorinated naphthenic acids | 55 |
| Chlorhexahydrobenzoic acid   |    |
| Chlorchaulmoogric acid       |    |
| Chlorhydrocarpic acid        | 65 |

When the second type of condensation reaction is employed, i. e., that identified under (2) above, where an aromatic acid is condensed with an aliphatic compound, the aromatic acid may be any of the acids given in Table I above.

When the condensation reaction of the type identified under (2) (a) above is employed, the unsaturated aliphatic compounds, which may be used in such condensation reaction, may be any of those listed in the following table.

TABLE VII.—*Unsaturated aliphatic compounds*

|    |                                                                                                                                                                                                                                                                                                                  |  |
|----|------------------------------------------------------------------------------------------------------------------------------------------------------------------------------------------------------------------------------------------------------------------------------------------------------------------|--|
| 5  | Ethylene                                                                                                                                                                                                                                                                                                         |  |
|    | Propylene                                                                                                                                                                                                                                                                                                        |  |
| 5  | Butylene                                                                                                                                                                                                                                                                                                         |  |
|    | Isobutylene                                                                                                                                                                                                                                                                                                      |  |
| 10 | Decene                                                                                                                                                                                                                                                                                                           |  |
|    | Acetylene                                                                                                                                                                                                                                                                                                        |  |
| 10 | Butadiene                                                                                                                                                                                                                                                                                                        |  |
|    | Allene                                                                                                                                                                                                                                                                                                           |  |
| 15 | Amylene                                                                                                                                                                                                                                                                                                          |  |
|    | As well as those unsaturated products derived from petroleum and petroleum fractions and derivatives such as paraffin wax as by cracking or for example removal of HCl by NaOH from monochlor paraffins. The unsaturated products derived from cracked gasoline, gas oil etc. will be found particularly useful. |  |

20 In the following table are listed a number of representative halogenated aliphatic compounds which may be used as one of the components of the condensation reaction identified under (2) (b) above.

TABLE VIII.—*Halogenated aliphatic compounds*

|    |                                                                                                                                                     |  |
|----|-----------------------------------------------------------------------------------------------------------------------------------------------------|--|
| 30 | Ethyl chloride                                                                                                                                      |  |
|    | Butyl chloride                                                                                                                                      |  |
| 30 | Amyl chloride                                                                                                                                       |  |
|    | Lauryl chloride                                                                                                                                     |  |
| 35 | Benzyl chloride                                                                                                                                     |  |
|    | Ethylene dichloride                                                                                                                                 |  |
|    | Carbon tetrachloride                                                                                                                                |  |
|    | Chlorparaffin wax                                                                                                                                   |  |
| 40 | Chlor naphtha                                                                                                                                       |  |
|    | Chlor decane                                                                                                                                        |  |
|    | Amyl dichloride                                                                                                                                     |  |
|    | Chlorinated aliphatic paraffin derivatives as well as the chlorinated derivatives of the various materials and compounds listed in Table VII above. |  |

45 In the following table are listed a number of specific examples of unsaturated cyclo-aliphatic compounds which may be employed as components of the condensation reaction identified under (2) (c) above.

TABLE IX.—*Unsaturated cyclo-aliphatic compounds*

|    |                |  |
|----|----------------|--|
| 50 | Cyclohexene    |  |
|    | Cyclohexadiene |  |
| 50 | Cyclopentene   |  |
|    | Cyclobutene    |  |

55 In the following table are listed a number of representative examples of halogenated cyclo-aliphatic compounds which may be employed as one of the components of the condensation reaction identified under (2) (d) above.

TABLE X.—*Halogenated cyclo-aliphatic compounds*

|    |                      |  |
|----|----------------------|--|
| 60 | Chlorcyclobutane     |  |
|    | Chlorcyclopentane    |  |
| 65 | Chlorehylcyclobutane |  |
|    | Chlorcyclohexane     |  |
|    | Dichlorcyclohexane   |  |
|    | Chlorcycloparaffin   |  |
|    | Chlorcyclopentane    |  |

70 The various aromatic acids, either those specifically identified in Table I above or those prepared by the various condensation reactions above identified, may, as previously indicated, be combined with either an organic radicle or base 75 in the preparation of organic salts or with in-

organic bases in the preparation of the inorganic salts.

In the following table will be found listed a number of organic radicles or bases which may thus be employed in the preparation of organic salts of aromatic acids.

TABLE XI.—*Organic radicles or bases*

Amino compounds such as:

|    |                  |  |
|----|------------------|--|
| 50 | Monoethanolamine |  |
|    | Diethanolamine   |  |
| 50 | Triethanolamine  |  |
|    | Aniline          |  |
| 55 | Benzylamine      |  |
|    | Laurylamine      |  |
|    | Diphenylamine    |  |
| 60 | Triphenylamine   |  |
|    | Diethylamine     |  |
| 65 | Triethylamine    |  |
|    | Putrescine       |  |

Nitrogen ring compounds, such as:

|     |              |  |
|-----|--------------|--|
| 65  | Pyrimidine   |  |
|     | Pyrazine     |  |
| 70  | Phenazine    |  |
|     | Quinazoline  |  |
| 75  | Pyrroline    |  |
|     | Pyridazine   |  |
| 80  | Picoline     |  |
|     | Pyrazole     |  |
| 85  | Pyridine     |  |
|     | Quinoline    |  |
| 90  | Pyrrole      |  |
|     | Piperidene   |  |
| 95  | Thiazole     |  |
|     | Carbazole    |  |
| 100 | Phenoxazine  |  |
|     | Phenthiazine |  |
| 105 | Indole       |  |
|     | Indoxyl      |  |
| 110 | Thiodiazole  |  |

Oxygen-bearing ring compounds, such as:

$\gamma$ -pyrone

Among the specific organic salts of aromatic acids which may thus be prepared for use, may be listed the following as illustrative examples.

TABLE XII.—*Organic salts*

|    |                                     |  |
|----|-------------------------------------|--|
| 50 | Aniline phenyl stearate             |  |
|    | Benzylamine chlorphenylstearate     |  |
| 55 | Laurylamine naphthylstearate        |  |
|    | Diphenylamine chlornaphthylstearate |  |
| 60 | Diethylamine phenylmercaptostearate |  |
|    | Ethanolamine phenylpalmitate        |  |
| 65 | Triethanolamine pipidyllaurate      |  |
|    | Pyridine phenyl stearate            |  |
| 70 | Quinoline naphthyl palmitate        |  |
|    | Piperidene chlor naphthyl laurate   |  |
| 75 | Thiazole phenyl palmitate           |  |
|    | $\gamma$ -pyrone phenyl stearate    |  |

In the following table are listed a number of inorganic radicles which may be combined with any of the aromatic acids given above in the production of inorganic salts of aromatic acids which may be used as addition agents in the lubricating compositions of my invention.

TABLE XIII.—*Inorganic radicles*

|    |           |  |
|----|-----------|--|
| 70 | Sodium    |  |
|    | Potassium |  |
| 75 | Ammonium  |  |
|    | Lithium   |  |
| 80 | Magnesium |  |
|    | Calcium   |  |

TABLE XIII.—*Inorganic radicles—Continued*

|     |                            |
|-----|----------------------------|
| 5.  | Strontium                  |
|     | Barium                     |
|     | Cobalt                     |
| 5.  | Zinc                       |
|     | Nickel                     |
|     | Manganese                  |
|     | Aluminum                   |
| 10. | Chromium                   |
|     | Stannous                   |
|     | Lead                       |
|     | Copper                     |
|     | Cadmium                    |
| 15. | Bismuth                    |
|     | Silver                     |
|     | Mercury                    |
|     | Vanadyl (VO <sub>3</sub> ) |

In the following table are given a list of 20 representative inorganic salts which may be produced by the combination of certain of the aromatic acids above identified with certain of the inorganic radicles of Table XIII above.

TABLE XIV.—*Inorganic salts*

|     |                                        |
|-----|----------------------------------------|
| 20. | Calcium diphenyl acetate               |
|     | Magnesium diphenyl acetate             |
|     | Nickel diphenyl acetate                |
| 30. | Cobalt diphenyl acetate                |
|     | Stannous diphenyl acetate              |
|     | Sodium phenyl stearate                 |
|     | Potassium phenyl stearate              |
|     | Ammonium phenyl stearate               |
| 35. | Lithium phenyl stearate                |
|     | Magnesium phenyl stearate              |
|     | Calcium phenyl stearate                |
|     | Strontium phenyl stearate              |
|     | Barium phenyl stearate                 |
| 40. | Cobalt phenyl stearate                 |
|     | Zinc phenyl stearate                   |
|     | Nickel phenyl stearate                 |
|     | Manganese phenyl stearate              |
|     | Aluminum phenyl stearate               |
| 45. | Chromium phenyl stearate               |
|     | Stannous phenyl stearate               |
|     | Copper phenyl stearate                 |
|     | Cadmium phenyl stearate                |
|     | Silver phenyl stearate                 |
| 50. | Vanadyl phenyl stearate                |
|     | Calcium phenyl mercapto stearate       |
|     | Magnesium phenyl mercapto stearate     |
|     | Nickel phenyl mercapto stearate        |
|     | Cobalt phenyl mercapto stearate        |
| 55. | Stannous phenyl mercapto stearate      |
|     | Calcium xenyl stearate                 |
|     | Magnesium xenyl stearate               |
|     | Nickel xenyl stearate                  |
|     | Cobalt xenyl stearate                  |
| 60. | Stannous xenyl stearate                |
|     | Calcium naphthyl stearate              |
|     | Magnesium naphthyl stearate            |
|     | Nickel naphthyl stearate               |
|     | Cobalt naphthyl stearate               |
| 65. | Stannous naphthyl stearate             |
|     | Calcium tolyl stearate                 |
|     | Magnesium tolyl stearate               |
|     | Nickel tolyl stearate                  |
|     | Cobalt tolyl stearate                  |
| 70. | Stannous tolyl stearate                |
|     | Magnesium butyl phthalate (salt-ester) |
|     | Calcium butyl phthalate (salt-ester)   |
|     | Nickel butyl phthalate (salt-ester)    |
|     | Cobalt butyl phthalate (salt-ester)    |
|     | Aluminum butyl phthalate (salt-ester)  |
| 75. | Calcium decyl phthalate (salt-ester)   |

TABLE XIV.—*Inorganic salts—Continued*

|     |                                                                                                                                                 |
|-----|-------------------------------------------------------------------------------------------------------------------------------------------------|
| 5.  | Cobalt decyl phthalate (salt-ester)                                                                                                             |
|     | Nickel decyl phthalate (salt-ester)                                                                                                             |
|     | Stannous decyl phthalate (salt-ester)                                                                                                           |
|     | Calcium lauryl phthalate (salt-ester)                                                                                                           |
|     | Cobalt lauryl phthalate (salt-ester)                                                                                                            |
|     | Nickel lauryl phthalate (salt-ester)                                                                                                            |
|     | Stannous lauryl phthalate (salt-ester)                                                                                                          |
|     | Magnesium mercapto rosolate                                                                                                                     |
| 10. | Calcium mercapto rosolate                                                                                                                       |
|     | Nickel mercapto rosolate                                                                                                                        |
|     | Cobalt mercapto rosolate                                                                                                                        |
|     | Aluminum mercapto rosolate                                                                                                                      |
| 15. | The halogen-bearing salts corresponding to the foregoing halogen-free salts will be found of utility and the following are particularly useful: |
|     | Calcium chlor phenyl stearate                                                                                                                   |
|     | Sodium chlor phenyl stearate                                                                                                                    |
|     | Magnesium chlor phenyl stearate                                                                                                                 |
| 20. | Calcium chlor naphthyl palmitate                                                                                                                |
|     | Stannous chlor phenyl palmitate                                                                                                                 |
|     | Calcium chlor phenyl laurate                                                                                                                    |
|     | Sodium chlor phenyl laurate                                                                                                                     |
|     | Nickel chlor phenyl laurate                                                                                                                     |
|     | Cobalt chlor phenyl laurate                                                                                                                     |
|     | Stannous chlor phenyl laurate                                                                                                                   |
|     | Calcium chlor phenyl palmitate                                                                                                                  |
|     | Sodium chlor phenyl palmitate                                                                                                                   |
| 25. | Nickel chlor phenyl palmitate                                                                                                                   |
|     | Cobalt chlor phenyl palmitate                                                                                                                   |
|     | Stannous chlor phenyl palmitate                                                                                                                 |
|     | Calcium chlor phenyl myristate                                                                                                                  |
|     | Sodium chlor phenyl myristate                                                                                                                   |
|     | Nickel chlor phenyl myristate                                                                                                                   |
| 30. | Cobalt chlor phenyl myristate                                                                                                                   |
|     | Stannous chlor phenyl myristate                                                                                                                 |
|     | Calcium chlor naphthyl laurate                                                                                                                  |
|     | Sodium chlor naphthyl laurate                                                                                                                   |
|     | Nickel chlor naphthyl laurate                                                                                                                   |
|     | Cobalt chlor naphthyl laurate                                                                                                                   |
|     | Stannous chlor naphthyl laurate                                                                                                                 |
|     | Calcium chlor naphthyl palmitate                                                                                                                |
|     | Sodium chlor naphthyl palmitate                                                                                                                 |
| 35. | Nickel chlor naphthyl palmitate                                                                                                                 |
|     | Cobalt chlor naphthyl myristate                                                                                                                 |
|     | Stannous chlor naphthyl myristate                                                                                                               |
|     | Calcium chlor xenyl laurate                                                                                                                     |
|     | Sodium chlor xenyl laurate                                                                                                                      |
|     | Nickel chlor xenyl laurate                                                                                                                      |
| 40. | Cobalt chlor xenyl laurate                                                                                                                      |
|     | Stannous chlor xenyl laurate                                                                                                                    |
|     | Calcium chlor xenyl palmitate                                                                                                                   |
|     | Sodium chlor xenyl palmitate                                                                                                                    |
|     | Nickel chlor xenyl palmitate                                                                                                                    |
| 45. | Cobalt chlor naphthyl palmitate                                                                                                                 |
|     | Stannous chlor naphthyl palmitate                                                                                                               |
|     | Calcium chlor naphthyl myristate                                                                                                                |
|     | Sodium chlor naphthyl myristate                                                                                                                 |
|     | Nickel chlor naphthyl myristate                                                                                                                 |
| 50. | Cobalt chlor naphthyl myristate                                                                                                                 |
|     | Stannous chlor naphthyl myristate                                                                                                               |
|     | Calcium chlor xenyl laurate                                                                                                                     |
|     | Sodium chlor xenyl laurate                                                                                                                      |
|     | Nickel chlor xenyl laurate                                                                                                                      |
| 55. | Cobalt chlor xenyl laurate                                                                                                                      |
|     | Stannous chlor xenyl laurate                                                                                                                    |
|     | Calcium chlor xenyl palmitate                                                                                                                   |
|     | Sodium chlor xenyl palmitate                                                                                                                    |
|     | Nickel chlor xenyl palmitate                                                                                                                    |
| 60. | Cobalt chlor xenyl palmitate                                                                                                                    |
|     | Stannous chlor xenyl palmitate                                                                                                                  |
|     | Calcium chlor xenyl myristate                                                                                                                   |
|     | Sodium chlor xenyl myristate                                                                                                                    |
|     | Nickel chlor xenyl myristate                                                                                                                    |
| 65. | Cobalt chlor xenyl myristate                                                                                                                    |
|     | Stannous chlor xenyl myristate                                                                                                                  |
|     | Calcium chlor tolyl laurate                                                                                                                     |
|     | Sodium chlor tolyl laurate                                                                                                                      |
|     | Nickel chlor tolyl laurate                                                                                                                      |
| 70. | Cobalt chlor tolyl laurate                                                                                                                      |
|     | Stannous chlor tolyl laurate                                                                                                                    |
|     | Calcium chlor tolyl palmitate                                                                                                                   |
|     | Sodium chlor tolyl palmitate                                                                                                                    |
|     | Nickel chlor tolyl palmitate                                                                                                                    |
| 75. |                                                                                                                                                 |

TABLE XIV.—*Inorganic salts*—Continued

|   |                                 |
|---|---------------------------------|
| 5 | Cobalt chlor toluyl palmitate   |
|   | Stannous chlor toluyl palmitate |
|   | Calcium chlor toluyl myristate  |
|   | Sodium chlor toluyl myristate   |
|   | Nickel chlor toluyl myristate   |
|   | Cobalt chlor toluyl myristate   |
|   | Stannous chlor toluyl myristate |

10 Salts of any of the metals of Table XIII with an aromatic acid produced by condensing paraffin wax hydrocarbons with benzoic acid. The salts produced by combining the metals of Table XIII with an aromatic acid such as with benzoic acid, 15 toluic acid or salicylic acid having one or more long aliphatic groups condensed onto the ring structure.

|    |                         |
|----|-------------------------|
| 20 | Calcium lauryl toluate  |
|    | Cobalt lauryl toluate   |
|    | Nickel lauryl toluate   |
|    | Stannous lauryl toluate |

Instead of preparing the salts designed for use as the addition agents of the present invention by treating any of the acids, of the type above identified, with an alkali for example such as sodium hydroxide in the preparation of the corresponding sodium salt of the acid, it is also possible to prepare corresponding salts by first preparing an ester of the acid, and then reacting such ester with an alkali such as sodium hydroxide to prepare, for example, the sodium soap of the acid, and then treating such soap with another salt in the preparation of a salt of a different inorganic radicle. Thus, for example, the methyl ester of chlorphenylstearic acid may be reacted with sodium hydroxide in the production of sodium chlorphenylstearate which is in turn reacted with calcium chloride in the production of calcium chlorphenyl stearate.

It may be preferable to prepare the ester, employed in the foregoing preparation of the salt, where such ester is one of an aromatic acid belonging to classification 2 on page 2 above, by condensing an ester of an aromatic acid with an unsaturated compound or halogenated organic compound instead of condensing the aromatic acid itself with such compound. For example, in the preparation of salts of stearoyl benzoic acid, methyl benzoate may be condensed with stearoyl chloride to form methyl stearoyl benzoate, this ester saponified with sodium hydroxide, and the resulting sodium salt reacted with magnesium chloride in aqueous solution to form magnesium stearoyl benzoate. An example of the preparation of magnesium stearoyl benzoate in detail is as follows:

A mixture of 1 mole each of methyl benzoate and stearoyl chloride is dissolved in an equal weight of carbon bisulphide. One mole of anhydrous aluminum chloride is added slowly with the temperature at 45° C. and the mixture held at that temperature for one hour longer. The materials are then poured into a mixture of cracked ice and concentrated hydrochloric acid, and the carbon bisulphide layer removed and washed with warm water. Carbon bisulphide and moisture are then removed by distilling under vacuum leaving the condensation product, namely 70 methyl stearoyl benzoate. The latter is saponified by adding 1 mole of sodium hydroxide in the form of a 10% aqueous solution, the mixture being refluxed until the aqueous solution is approximately neutral. One-half mole of magnesium chloride is added in the form of an aqueous

solution which causes the precipitation of magnesium stearoyl benzoate. The water layer is decanted from the precipitate which is then dissolved in benzol and dried by removing the benzol and water by distilling under vacuum. The resulting product was dissolved in a naphthenic type oil in a concentration of 1% and found to materially improve the oil when used in an internal combustion engine, particularly in preventing the formation of harmful deposits on the 10 piston and piston rings.

Included among the compounds contemplated for use by this invention are stable oil soluble salt-esters of polybasic aromatic acids. These may be formed for example by neutralizing an acid ester of a polybasic aromatic acid with a base, or by partially saponifying a neutral ester of a polybasic aromatic acid with a base so that each molecule of the saponified material retains at least one ester group in addition to at least one basic group.

Examples of such compounds are the salt-esters of the following:

|                                            |    |
|--------------------------------------------|----|
| 1. Benzene polycarboxylic acids, e. g.     | 25 |
| Phthalic acids                             |    |
| Trimesic acid                              |    |
| Trimellitic acid                           |    |
| Hemimellitic acid                          |    |
| Pyromellitic acid                          | 30 |
| Mellophanic acid                           |    |
| Prehnitic acid                             |    |
| Benzene pentacarboxylic acid               |    |
| 2. Naphthalene polycarboxylic acids, e. g. | 35 |
| Naphthalic acids                           |    |
| 3. Pyridine polycarboxylic acids, e. g.    | 40 |
| Lutidinic acid                             |    |
| Dipicolinic acid                           |    |
| Cynchomeronic acid                         |    |
| Isocynchomeronic acid                      |    |
| Dinicotinic acid                           |    |
| Alpha-carbocynchomeronic acid              | 45 |
| Beta-carbocynchomeronic acid               |    |
| Berberonic acid                            |    |
| Trimesitinic acid                          |    |
| Pyridine tetracarboxylic acid              |    |
| Pyridine pentacarboxylic acid              |    |
| 4. Pyrrole polycarboxylic acids            | 50 |
| 5. Quinoline polycarboxylic acids          |    |
| 6. Thiophene polycarboxylic acids          |    |
| 7. Thiazole polycarboxylic acids           |    |
| 8. Diphenyl polycarboxylic acids, e. g.    | 55 |
| Diphenic acid                              |    |
| 9. Dibenzyl polycarboxylic acids           |    |
| 10. Anthracene polycarboxylic acids        |    |
| 11. Phenanthrene polycarboxylic acids      |    |
| 12. Thianthrene polycarboxylic acids       |    |

Where such salt-esters are employed, it will generally be found advantageous to have at least one of the ester groups consist of an aliphatic or cyclo-aliphatic group and preferably one containing four or more carbon atoms. For example, salts of the acid butyl or amyl esters of phthalic acid have been found suitable.

Specific examples of these salt-esters have been 65 labeled in the principal list of specific examples given above.

In view of the particular uses for which my compounded lubricants are intended, it is apparent that of the salts included in the foregoing 70 enumeration of the addition agents which may be employed, those which are readily oil-soluble are the ones preferred for use. When these compounded oils are designed for use under conditions where high temperatures are usually en- 75

countered, the addition agents should be stable at elevated temperatures. For use in crankcase lubricants for internal combustion engines, they should preferably be stable to the extent where 5 there will be substantially no decomposition, when the lubricating composition is exposed to temperatures up to 250° F.

The addition agents which are to be selected from the class described should be such that they 10 are relatively non-corrosive with respect to the metallic surfaces with which they come in contact during use. Certain of the named addition agents may be found to be detrimentally corrosive to certain sensitive bearing metals, in 15 which case an appropriate corrosion inhibitor may be employed in conjunction therewith in the composition.

A lubricating composition prepared in accordance with my invention and which is predominantly hydrocarbon oil may contain from an effective amount to 20% of the salt addition agent above identified. In general, it will be found that an amount as low as 1% will often be quite effective and that amounts in excess of 10% are 25 seldom necessary. A preferred range of concentrations for the salt in the oil is from .25% to about 2%.

It is also within the contemplation of this invention to provide the addition agents in the form 30 of a concentrate in a suitable oil, said oil containing rather high percentages of the addition agents. Such concentrates may be employed for further blending with a lubricating oil in the proportions desired for the particular conditions 35 of use.

While mineral oil, generally, is the principal ingredient of the lubricant, it is not essential that it be the only ingredient other than the addition agents, provided that there be no additional 40 ingredient which is incompatible with such addition agent. It is within the contemplation of this invention to include, if necessary or desirable, such other addition agents as are commonly added to improve the viscosity index or 45 cold test of the lubricants; and a lubricating composition according to this invention which also has a separate film-strength or oiliness increasing agent has been found to be especially effective.

50 When used in conjunction with a hydrocarbon lubricating oil, it is obvious that, generally, only such amounts of the addition agent may be included as are soluble in the specified amount of oil. By the term "soluble," as herein used, it is 55 intended to indicate the ability to form not only true solutions but also any form of substantially permanently homogeneous composition when incorporated in mineral oil. With most of the compounds there is usually little difficulty, especially 60 if the incorporation is effected in the manner described in Cornell Patent No. 2,042,880, and since quite small percentages often give remarkably improved results, it is seldom of extreme importance that the addition agents be oil-soluble in all proportions. Also, certain compounds are of value 65 as gelling or bodying agents when used in amounts greater than are strictly soluble.

The addition agents above enumerated for use 70 in my compounded lubricants include certain ones which may be found to at least partially decompose under conditions of extreme stress such as the very high temperature encountered in certain classes of use, while others are quite stable even under such extreme conditions.

75 The use for which the lubricant is designed

therefore determines the particular type of addition agent to be selected. A certain amount of decomposition, which proceeds at a relatively slow rate, is usually not harmful. Care should be exercised, however, to select for a particular set of 5 operating conditions, an addition agent which in the oil base used, will not decompose under such operating conditions except at a low rate.

By the term "stable" as used herein in describing the addition agents is meant the characteristic of the addition agents which enables them to resist decomposition in the oil under the condition of use for which the lubricating composition is designed.

The lubricating compositions of this invention 15 may be prepared by first preparing the salt and then dissolving the salt in the oil base, or they may be prepared by reacting the acid in solution in all or a portion of the oil with a suitable basic compound in order to form the desired salt directly in solution in oil. In the latter case, it is frequently desirable to remove the water formed by the reaction, or which may have been added with the basic compound, by some means such as by heating at atmospheric or sub-atmospheric 25 pressure.

In case the salt to be used is water-insoluble, an alternative procedure is as follows:

An aqueous solution of a water-soluble salt of the acid is first prepared, for example by dissolving the acid in an aqueous solution of caustic soda or caustic potash. The aqueous salt solution is then emulsified with oil and a water-soluble salt containing the cation of the desired salt is added to the mixture. The desired salt is thus precipitated from the aqueous medium and subsequently or simultaneously dissolved by the oil medium. Separation of the aqueous and oil layers is then effected for example by settling or centrifuging. Subsequent water-washing of the oil solution to 40 remove traces of inorganic salts may be desirable, and removal of moisture may also be required.

It will be observed that all of the specific examples of addition agents for use in my improved lubricating composition may be defined as salts 45 of aromatic acids, which salts contain the radicle

-C-X-M

in which X is an element of the class consisting of 50 oxygen and sulphur and M is a member of the class consisting of metals and basic radicles.

This application is a continuation-in-part of my aforesaid co-pending applications Serial 55 Numbers 737,070, 216,153 and 245,226.

Other modes of applying the principle of the invention may be employed, change being made as regards the details described, provided the features stated in any of the following claims or the equivalent of such be employed.

I therefore particularly point out and distinctly claim as my invention:

1. A lubricating composition containing as a principal lubricating constituent a major amount of a mineral lubricating oil with the properties of 65 such composition affecting its use as a lubricant improved by incorporating therein a minor amount of a stable oil-soluble salt of an aromatic acid which salt contains the radicle

-C-X-M

in which X is an element of the class consisting of 70 oxygen and sulphur and M is a member of the class consisting of metals and basic radicles.

- 5 2. A lubricating composition containing as a principal lubricating constituent a major amount of a mineral lubricating oil with the properties of such composition affecting its use as a lubricant improved by incorporating therein a minor amount of a stable oil-soluble metallic salt of an aromatic acid which salt contains the radicle



10

in which **X** is an element of the class consisting of oxygen and sulphur and **M** is a member of the class consisting of metals and basic radicles.

- 15 3. A lubricating composition containing as a principal lubricating constituent a major amount of a mineral lubricating oil with the properties of such composition affecting its use as a lubricant improved by incorporating therein a minor amount of a stable oil-soluble halogen bearing salt of an aromatic acid.

20

25 4. A lubricating composition containing as a principal lubricating constituent a major amount of a mineral lubricating oil with the properties of such composition affecting its use as a lubricant improved by incorporating therein a minor amount of a stable oil-soluble halogen bearing metallic salt of an aromatic acid.

- 30 5. A lubricating composition containing as a principal lubricating constituent a major amount of a mineral lubricating oil with the properties of such composition affecting its use as a lubricant improved by incorporating therein a minor amount of a stable oil-soluble salt of a halogenated aromatic acid.

35 6. A lubricating composition containing as a principal lubricating constituent a major amount of a mineral lubricating oil with the properties of such composition affecting its use as a lubricant improved by incorporating therein a minor amount of a stable oil-soluble salt of an alkylated aromatic acid.

7. A lubricating composition containing as a principal lubricating constituent a major amount of a mineral lubricating oil with the properties of such composition affecting its use as a lubricant improved by incorporating therein a minor amount of a stable oil-soluble metallic salt of an alkylated aromatic acid.

8. A lubricating composition containing as a  
50 principal lubricating constituent a major amount  
of a mineral lubricating oil with the properties of  
such composition affecting its use as a lubricant  
improved by incorporating therein a minor  
55 amount of a stable oil-soluble halogen bearing  
metallic salt of an alkylated aromatic acid.

9. A lubricating composition containing as a principal lubricating constituent a major amount of a mineral lubricating oil with the properties of such composition affecting its use as a lubricant improved by incorporating therein a minor amount of a stable oil-soluble salt of an aromatic acid containing a substituent selected from the class consisting of aliphatic and cyclo-aliphatic radicles.

65 10. A lubricating composition containing as a principal lubricating constituent a major amount of a mineral lubricating oil with the properties of such composition affecting its use as a lubricant improved by incorporating therein a minor amount of a stable oil-soluble salt of an aromatic acid containing an aliphatic substituent.

- acid containing an aliphatic substituent.

11. A lubricating composition containing as a principal lubricating constituent a major amount of a mineral lubricating oil with the properties  
75 of such composition affecting its use as a lubri-

cant improved by incorporating therein a minor amount of a stable oil-soluble salt of an aromatic acid containing a cyclo-aliphatic substituent.

12. A lubricating composition containing as a principal lubricating constituent a major amount of a mineral lubricating oil with the properties of such composition affecting its use as a lubricant improved by incorporating therein a minor amount of a stable oil-soluble metallic salt of an aromatic acid containing a substituent selected from the class consisting of aliphatic and cyclo-aliphatic radicles. 5 10

13. A lubricating composition containing as a principal lubricating constituent a major amount of a mineral lubricating oil with the properties of such composition affecting its use as a lubricant improved by incorporating therein a minor amount of a stable oil-soluble metallic salt of an aromatic acid containing an aliphatic substituent.

14. A lubricating composition containing as a principal lubricating constituent a major amount of a mineral lubricating oil with the properties of such composition affecting its use as a lubricant improved by incorporating therein a minor amount of a stable oil-soluble metallic salt of an aromatic acid containing a cyclo-aliphatic substituent.

15. A Lubricating composition containing as a principal lubricating constituent a major amount of a mineral lubricating oil with the properties of such composition affecting its use as a lubricant improved by incorporating therein a minor amount of a stable oil-soluble divalent metallic salt of an aromatic acid containing a substituent selected from the class consisting of aliphatic and cyclo-aliphatic radicles. 30 35

16. A lubricating composition containing as a principal lubricating constituent a major amount of a mineral lubricating oil with the properties of such composition affecting its use as a lubricant improved by incorporating therein a minor amount of a stable oil-soluble, halogen bearing salt of an aromatic acid containing a substituent selected from the class consisting of aliphatic and cyclo-aliphatic radicles. 40 45

17. A lubricating composition containing as a principal lubricating constituent a major amount of a mineral lubricating oil with the properties of such composition affecting its use as a lubricant improved by incorporating therein a minor amount of a stable oil-soluble, halogen bearing metallic salt of an aromatic acid containing a substituent selected from the class consisting of aliphatic and cyclo-aliphatic radicles. 50 56

18. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic acid with an unsaturated aliphatic compound. 60

19. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing a halogenated aromatic acid with an unsaturated, aliphatic compound.

20. A lubricating composition containing as a principal lubricating constituent a major amount 75

- of a mineral lubricating oil with the properties of such composition affecting its use as a lubricant improved by incorporating therein a minor amount of a stable oil-soluble salt of an aromatic acid of the type which may be produced by condensing an aromatic acid with a halogenated aliphatic compound.
21. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic acid with an unsaturated cyclo-aliphatic compound.
22. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic acid with a halogenated cyclo-aliphatic compound.
23. A lubricating composition containing as a principal lubricating constituent a major amount of a mineral lubricating oil with the properties of such composition affecting its use as a lubricant improved by incorporating therein a minor amount of a stable oil-soluble salt
- of an aromatic acid of the type which may be produced by condensing an aromatic compound with an unsaturated aliphatic acid.
24. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic compound with a halogenated aliphatic acid.
25. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic compound with an unsaturated cyclo-aliphatic acid.
26. A lubricating composition containing as a principal lubricating constituent a major amount of a mineral lubricating oil with the properties of such composition affecting its use as a lubricant improved by incorporating therein a minor amount of a stable oil-soluble salt of an aromatic acid of the type which may be produced by condensing an aromatic compound with a halogenated cyclo-aliphatic acid.

CARL F. PRUTTON.